

# United States Patent [19]

Okada et al.

[11] 3,929,472

[45] Dec. 30, 1975

[54] STEEL SHEETS HAVING EXCELLENT RUST RESISTANCE

[75] Inventors: **Hideya Okada**, Yokohama; **Haruo Shimada**, Tokyo, both of Japan

[73] Assignee: **Nippon Steel Corporation**, Tokyo, Japan

[22] Filed: **Dec. 19, 1974**

[21] Appl. No.: **534,579**

## Related U.S. Application Data

[63] Continuation of Ser. No. 358,305, May 8, 1973, abandoned.

## Foreign Application Priority Data

May 11, 1972 Japan..... 47-46648  
July 8, 1972 Japan..... 47-67889  
Mar. 31, 1973 Japan..... 48-27120

[52] U.S. Cl. .... **75/124; 75/123 E; 75/126 D; 75/126 G; 75/126 P; 75/128 E; 75/128 F; 75/128 T**

[51] Int. Cl.<sup>2</sup> ..... **C22C 38/00**

[58] **Field of Search**..... 75/123 E, 124, 125, 126 D, 75/126 G, 126 P, 128 E, 128 F, 128 T

## [56] References Cited UNITED STATES PATENTS

|           |         |                       |          |
|-----------|---------|-----------------------|----------|
| 2,861,908 | 11/1958 | Mickelson et al.....  | 75/128 E |
| 3,310,441 | 3/1967  | Mandich.....          | 148/36   |
| 3,711,340 | 1/1973  | Korchynsky et al..... | 75/124   |

*Primary Examiner*—L. Dewayne Rutledge  
*Assistant Examiner*—Arthur J. Steiner  
*Attorney, Agent, or Firm*—Toren, McGeady and Stanger

## [57] ABSTRACT

A steel sheet having excellent rust and corrosion resistance, comprising 0.001-0.15% C, 0.01-1.04% Si, 0.01-1.0% Mn, 0.001-0.05% Al, 0.01-0.5% Cu, 0.001-0.04% P, 0.002-0.07% S and Ce in an amount to maintain the weight ratio of Ce/S between 0.1-50, with the balance being iron and unavoidable impurities.

**3 Claims, 2 Drawing Figures**

FIG.1



FIG.2



## STEEL SHEETS HAVING EXCELLENT RUST RESISTANCE

This is a continuation of application Ser. No. 358,305 filed May 8, 1973 now abandoned.

The present invention relates to steel sheets having excellent rust and corrosion resistance suitable for automobile parts and can-making. Conventionally, during the production process or during transportation to users, these steel sheets have been often damaged by rust formation, and clarification of its causes and appropriate measures therefore have been sought for by the steel maker, and improvement of corrosion resistance, in addition of prevention of the rust formation has been demanded by users particularly for making Coca Cola cans.

The present inventors have conducted extensive studies on causes of rust formation to find measures to satisfy the above two demands, and as the result it has been found for the first time that the rust formation on commercial steels develops in the following process, and this process of rust formation has been clarified by a unique method for determining the physical properties of sulfides present in the steel (the sulfides are separated by electrolytic extraction to clarify their physical properties, for example their solubility in water, etc.). The process of rust formation on commercial steels progresses as under.

When dews are formed on the steel sheet, first sulfides  $\alpha$  (Mn, Fe) S present in the steel are dissolved into the dews, and then dissolved  $Mn^{++}$  and  $Fe^{++}$  are oxidized by oxygen in water and  $Mn^{+++}$  and  $Fe^{+++}$  precipitate as  $2Mn_2O_3$  and  $FeOOH$ , which act as nuclei for formation of  $\gamma Mn_2O_3$ .

Then, the thus formed  $\gamma Mn_2O_3$  is dispersed rapidly on the steel surface as colloidal particles and also settles as dispersed colloids around  $\alpha$  (Mn, Fe) S which has not yet taken remarkable change so that ring-like sediments settle around  $\alpha$  (Mn, Fe) S or original  $\alpha$  (Mn, Fe) S. These sediments easily adsorb water and thus causes subsequent wet corrosion reaction and results in the formation of red rust of  $\gamma FeOOH$ . Therefore, in order to prevent or reduce such rust formation, it is necessary to reduce the sulfur content in the steel as low as possible so as to reduce  $\alpha$  (Mn, Fe) S content in the steel. However, it takes considerable expense to reduce the sulfur content in the steel and yet it is impossible to reduce the sulfur content to zero. Therefore, other measures must be taken to reduce or prevent the formation of  $\alpha$  (Mn, Fe) S. What is the most important in the process of rust formation is the fact that  $\alpha$  (Mn, Fe) S is soluble in water. Therefore, the rust formation can be prevented by a primitive method such as by changing the physical properties of  $\alpha$  (Mn, Fe) S or by converting this sulfide into other metal sulfide which hardly reacts with water.

From the above point of view, the present inventors have studied the dissolution behaviour of various sulfides into water, and the results are shown in FIG. 1. These sulfides were separated by electrolytically extraction from hot rolled steel plates containing various metals such as Ce, V, Ti, Mn and sulfur. It is understood from FIG. 1 that the dissolution behaviour into water varies remarkably depending on the kind and type of sulfides.

On the other hand, when the steel sheet is used for Cola beverage cans, it is necessary to increase the sul-

fur content in the steel and retain the dissolved  $SH^-$  ion in the beverage in order to increase the corrosion resistance. Therefore, for this purpose it is necessary the sulfide present in the steel dissolves into the Cola beverage contrary to the case of improving the rust resistance.

The  $\alpha$  (Mn, Fe) S commonly present in commercial steels dissolves in the Cola beverage as well as in water and thus this sulfide is favourable to corrosion resistance in the Cola cans although is not desirable for rust resistance.

The present invention will be described by referring to the attached drawings.

FIG. 1 is a graph showing dissolution behaviours of various sulfides electrolytically extracted from the steel when immersed in water (air saturated) at different temperatures for 20 minutes; and

FIG. 2 is a graph showing dissolution behaviours of the same sulfides when immersed in the blue dye solution ( $CO_2$  atmosphere) for 10 hours.

There are certain sulfides which hardly dissolves in water and at the same time it hardly dissolves in a liquid having pH value of 2-3 such as the Cola beverage. Therefore, the present inventors have studies the dissolution behaviour of the various sulfides as mentioned before in a blue dye solution simulated to the Cola beverage. The results are shown in FIG. 2. It is understood from FIG. 2 that the dissolution behaviour in the blue dye solution varies remarkably depending on the kind and type of the sulfides. Based on the results shown in FIG. 1 and FIG. 2, the present inventors have developed steel sheets having excellent rust resistance, and further developed steel sheets suitable for carbonate beverage cans such as Cola cans and steel sheets suitable for beer cans by adjusting the properties of the sulfide.

The base steel composition according to the present invention comprises 0.001-0.15% of C, 0.01-1.0% of Si, 0.01-1.0% of Mn, 0.001-0.05% of Al, 0.01-0.5% of Cu, 0.001-0.04% of P, 0.002-0.07% of S with addition of Ce in an amount so as to maintain the weight ratio of Ce/S between 0.1-5.0, with the balance being iron and unavoidable impurities. The basic components of the above composition are iron, carbon, manganese, copper, cerium and sulfur, and these elements are called as the first group elements.

Next, the basic steel composition may contain one or more of Cr, B, Ni and Ti in addition to the above elements and these elements are called as the second group elements.

In the first group elements, cerium, when present with copper, contributes to improve the rust resistance and particularly when the weight ratio of Ce/S is between 0.1-50, remarkable rust resistance as well as remarkable corrosion resistance in the blue dye solution are obtained.

The elements in single of the second group tend to improve the rust resistance and sometimes further improve the rust resistance when the first group elements are present with the second group elements.

Thus the modified steel composition of the present invention comprises 0.001-0.15% of C, 0.01-1.0% of Si, 0.01-1.0% of Mn, 0.001-0.05% of Al, 0.01-0.5% of Cu, 0.002-0.07% of S, with addition of Ce in an amount so as to maintain the weight ratio of Ce/S between 0.1-50, and if necessary one or more 0.005-1.0% of Cr, 0.05-1.0% of Ni, 0.001-0.05% of B, and 0.001-0.1% of Ti.

A further modified steel composition of the present invention comprises three or more of V, Zr, Pr, Nd and Y in an amount between 0.05-0.7 in total, corresponding to 0.2-30% of the sulfur content, with the balance being iron and unavoidable impurities.

The above ranges for individual elements in the present invention have been decided as effective ranges from the points of corrosion resistance mechanical properties and steel-making aspects. Thus, carbon is necessary for obtaining required strength of the present inventive steel, but more than 0.15% of carbon lowers the elongation and deteriorates the rust resistance and less than 0.001% of carbon lowers the strength and elongate the steel refining time, thus deteriorates economical aspect and productivity. Silicon and manganese are necessary as deoxidizing element in the steel making process, more than 0.01% of each of Si and Mn, is required, but their excessive contents embrittle the steel and give excessive strength. Thus, their upper limit is set as 1.0% and their preferable ranges for Si and Mn are not less than 0.03% and not less than 0.3% respectively. Aluminium is sometimes added as deoxidizing element and for other purposes. Excessive addition of aluminium often forms much inclusions which causes steel defects and its upper limit is set at 0.05%. Cu is effective to promote rust resistance in cooperation with other elements, but less than 0.01% of Cu is not effective and more than 0.50% of Cu embrittles the steel and deteriorates the workability of the steel. Regarding phosphorus, it is desirable to restrict phosphorus as low as possible, and the range of 0.001-0.04% is defined by considering economical restrictions in the steel making process. It is also desirable to maintain the sulfur content as low as possible but the range of 0.002-0.07% is defined by considering economical restrictions in the steel making process. Cerium fixes sulfur as cerium sulfide or complex sulfide with other metal, and forms sulfides soluble in the blue dye solution. Thus the cerium content is so limited that the weight ratio of Ce/S is between 0.1-50. Cerium is usually accompanied with rare earth group elements such as lanthanum and, therefore, the present invention covers in its scope the case when cerium contains rare earth group elements such as lanthanum. The content of chromium as optional element is limited to 0.005-1.0% because the effect on rust resistance enhancement by chromium becomes remarkable when chromium is present more than 0.005%, by with chromium contents more than 1.0% increase the production cost. The boron range of 0.001-0.05% is decided because less than 0.001% of boron is not effective, but more than 0.05% of boron causes embrittlement of the steel. The nickel content is limited to 0.01-1.0% for the reason that the effect of rust resistance improvement by nickel becomes remarkable when nickel is present more than 0.01%, but nickel addition more than 1.0% increases production cost. The titanium range of 0.001-0.1% corresponds to the titanium amount remaining in the steel in case of Al-deoxidization or Ti deoxydization alone.

Three or more of V, Zr, Pr, Nd and Y are added for the reason that such addition provides steel sheets having excellent rust resistance as well as excellent corro-

sion resistance in carbonate beverage and beer etc. Namely by the addition of three or more of the above elements it is possible that unique sulfides which assure the required properties of the steel sheet, or spherical complex sulfides which hardly dissolve in water but dissolve into the blue dye are present in the steel. The content of the above elements and the ratio of the content of these elements to the sulfur content are adjusted so as to maintain the rust formation rate less than 20% by the Q.C. tester (explained hereinafter) to maintain the corrosion rate less than 50 $\mu$ A/cm in the blue dye solution by the simulate test for determining the rust resistance in the cola beverage, and to maintain the metal loss by corrosion in NaCl-citric acid solution by the beer can simulation test less than 0.30mg/cm. Thus, in the present invention, three or more of V, Zr, Pr, Nd, Y are added in an amount between 0.05-0.7% in total, and the sulfur content is adjusted to less than 0.07% so that the ratio of the total content to the sulfur content is between 0.2-30. The steel sheet of the above chemical composition according to the present invention is made by melting the starting steel material in an ordinary steel making furnace such as an electric furnace and a converter, using, if necessary, the vacuum degassing, making ingots by a continuous casting method or an ordinary ingot making method, hot rolling, cold rolling, and annealing (including continuous annealing). As the cases demand, the present inventive steel sheet may be used in "as hot rolled", "as hot rolled and normalized or annealed" or "as cold rolled" condition. Further, the present inventive steel sheet may be used as a substrate for surface treated steel sheet.

Examples of the present invention will be set forth under.

Table 1 shows the chemical compositions of the present inventive steels and conventional steels, both melted in a converter, cast into ingots, hot rolled, cold rolled and annealed. Table 2 shows results of corrosion resistance tests. In particular, Table 2 shows the surface condition (A<sub>1</sub>) after 3 months indoor exposure of the cold rolled annealed sheet, the rust formation (A<sub>2</sub>) by the Q.C. tester (dried for 15 minutes, wetted for 45 minutes, maintained for 16 hours with the outer surface at 20°C, the inside surface at 32°C and forming dews on the inside surface) the rust resistance (B) (blue-dye value) in the blue-dye solution, and the rust resistance (C) in the citric acid - NaCl solution. Also the surface conditions after 3 months indoor exposure of cold rolled steel sheets are shown in Table 2.

(A) in the table represents the ratio (%) of rust formation to surface for test pieces of 3mm thickness, 30mm width and 50mm length, (B) represents weight losses after 4 day immersion in 500 ml blue dye solution (CO<sub>2</sub> atmosphere) of 8cm<sup>2</sup> test pieces, and (C) represents weight losses after 4 day immersion in 500 ml citric acid - NaCl solution of 8cm<sup>2</sup> test pieces.

It is clearly understood from the results of (A), (B) and (C) in Table 2 that the present inventive steel sheets have remarkably excellent rust resistance and corrosion resistance as carbonate beverage cans and beer cans as compared with the conventional steels.

Table 1

| No.     | C | Si   | Mn   | Al  | Chemical Composition (%) |       |    |        |
|---------|---|------|------|-----|--------------------------|-------|----|--------|
|         |   |      |      |     | Ce                       | S     | Cu | Others |
| Conven- | 1 | 0.06 | 0.03 | 0.4 |                          | 0.010 |    |        |

Table 1-continued

| No.                      | C        | Si   | Mn   | Al    | Chemical Composition (%) |       |      | Others                            |
|--------------------------|----------|------|------|-------|--------------------------|-------|------|-----------------------------------|
|                          |          |      |      |       | Ce                       | S     | Cu   |                                   |
| tional<br>Steels         | 2 0.05   | 0.03 | 0.2  |       | 0.018                    |       |      |                                   |
|                          | 3 0.03   | 0.05 | 0.3  |       | 0.020                    |       | 0.15 |                                   |
| Inven-<br>tive<br>Steels | 4 0.02   | 0.01 | 0.10 | 0.002 | 0.02                     | 0.003 | 0.20 |                                   |
|                          | 5 0.01   | 0.02 | 0.10 | 0.003 | 0.03                     | 0.002 | 0.25 |                                   |
|                          | 6 0.03   | 0.01 | 0.15 | 0.005 | 0.02                     | 0.005 | 0.20 |                                   |
|                          | 7 0.01   | 0.01 | 0.17 | 0.003 | 0.02                     | 0.015 | 0.20 | La 0.005                          |
|                          | 8 0.02   | 0.01 | 0.16 | 0.005 | 0.02                     | 0.020 | 0.23 | La 0.01                           |
|                          | 9 0.01   | 0.02 | 0.20 | 0.006 | 0.05                     | 0.003 | 0.18 | Cr 0.03                           |
|                          | 10 0.02  | 0.01 | 0.10 | 0.005 | 0.02                     | 0.003 | 0.03 | Cr 1.0                            |
|                          | 11 0.005 | 0.01 | 0.10 | 0.005 | 0.07                     | 0.003 | 0.03 | Ti 0.003                          |
|                          | 12 0.005 | 0.01 | 0.10 | 0.005 | 0.07                     | 0.003 | 0.20 | B 0.005                           |
|                          | 13 0.02  | 0.01 | 0.15 | 0.01  | 0.03                     | 0.003 | 0.03 | Ni 0.3                            |
|                          | 14 0.02  | 0.01 | 0.15 | 0.02  | 0.05                     | 0.020 | 0.20 | Cr 0.8, B 0.006                   |
|                          | 15 0.01  | 0.01 | 0.15 | 0.01  | 0.02                     | 0.002 | 0.03 | Ti 0.003, Cr 0.03                 |
|                          | 16 0.01  | 0.01 | 0.15 | 0.01  | 0.02                     | 0.003 | 0.20 | V 0.05, Nd 0.005                  |
|                          | 17 0.01  | 0.01 | 0.15 | 0.01  | 0.02                     | 0.003 | 0.20 | V 0.03, Zr 0.02, Pr 0.005         |
|                          | 18 0.01  | 0.02 | 0.15 | 0.005 | 0.02                     | 0.003 | 0.15 | Cr 0.03, V 0.05, Pr 0.005, Y 0.06 |

Table 2

|    | Rust Formation<br>after 3 months<br>indoor exposure |                                      | Rust formation<br>determined by<br>Q.C. tester<br>% | Corrosion<br>rate in<br>blue dye<br>solution<br>( $\mu\text{A}/\text{cm}^2$ ) | Corrosion<br>rate in<br>citric acid<br>NaCl solu-<br>tion (mg/cm $^2$ ) |
|----|-----------------------------------------------------|--------------------------------------|-----------------------------------------------------|-------------------------------------------------------------------------------|-------------------------------------------------------------------------|
|    | cold<br>rolled<br>sheet                             | cold rolled<br>and<br>annealed sheet |                                                     |                                                                               |                                                                         |
| 1  | 100                                                 | 100                                  | 100                                                 | 60                                                                            | 1.1                                                                     |
| 2  | 100                                                 | 100                                  | 100                                                 | 45                                                                            | 1.0                                                                     |
| 3  | 80                                                  | 86                                   | 90                                                  | 47                                                                            | 0.5                                                                     |
| 4  | 10                                                  | 15                                   | 10                                                  | 17                                                                            | 0.30                                                                    |
| 5  | 8                                                   | 13                                   | 11                                                  | 17                                                                            | 0.30                                                                    |
| 6  | 8                                                   | 8                                    | 10                                                  | 30                                                                            | 0.30                                                                    |
| 7  | 7                                                   | 8                                    | 8                                                   | 10                                                                            | 0.28                                                                    |
| 8  | 7                                                   | 10                                   | 10                                                  | 15                                                                            | 0.15                                                                    |
| 9  | 6                                                   | 10                                   | 8                                                   | 11                                                                            | 0.18                                                                    |
| 10 | 7                                                   | 11                                   | 13                                                  | 7                                                                             | 0.30                                                                    |
| 11 | 12                                                  | 18                                   | 15                                                  | 8                                                                             | 0.25                                                                    |
| 12 | 7                                                   | 15                                   | 15                                                  | 11                                                                            | 0.20                                                                    |
| 13 | 5                                                   | 8                                    | 10                                                  | 10                                                                            | 0.18                                                                    |
| 14 | 10                                                  | 12                                   | 8                                                   | 15                                                                            | 0.28                                                                    |
| 15 | 10                                                  | 10                                   | 7                                                   | 11                                                                            | 0.25                                                                    |
| 16 | 8                                                   | 7                                    | 7                                                   | 10                                                                            | 0.17                                                                    |

What is claimed is:

1. A steel sheet having excellent rust and corrosion resistance, consisting of 0.001-0.15% C, 0.01-1.04% Si, 0.01-1.0% Mn, 0.001-0.05% Al, 0.01-0.5% Cu, 0.001-0.04% P, 0.002-0.07% S and Ce in an amount to maintain the weight ratio of Ce/S between 0.1-50, with the balance being iron and unavoidable impurities.

2. A steel sheet having excellent rust and corrosion resistance consisting of 0.001-0.15% carbon, 0.01-1.04% silicon, 0.01-1.0% manganese, 0.001-0.05% aluminum, 0.01-0.5% copper, 0.001-0.04% phosphorus, 0.002-0.07% sulfur, and cerium in an amount to maintain the weight ratio of cerium to sulfur between 0.1-50, and one or more elements selected from the group consisting of 0.005-1.0% chromium, 0.01-1.0% nickel,

0.001-0.05% boron, and 0.001-0.1% titanium, with the balance being iron and unavoidable impurities.

3. A steel sheet having excellent rust and corrosion resistance consisting of 0.001-0.15% carbon, 0.01-1.04% silicon, 0.01-1.0% manganese, 0.001-0.05% aluminum, 0.01-0.5% copper, 0.001-0.04% phosphorus, 0.002-0.07% sulfur, and cerium in an amount to maintain the weight ratio of cerium to sulfur between 0.1-50, and three or more elements selected from the group consisting of V, Z, Pr, Nd, and Y, in a total amount between 0.05-0.7%, the ratio of said total amount to the sulfur content being from 0.2-30, with the balance being iron and unavoidable impurities.

\* \* \* \* \*